

## UNITED STATES PATENT OFFICE.

WILLIAM FELDENHEIMER, OF LONDON, ENGLAND.

## TREATMENT OF CLAY.

No Drawing. Application filed June 16, 1925, Serial No. 37,467, and in Great Britain August 7, 1924.

The present invention relates to the treatment of clays for their purification and the improvement of their colour, the present application being a continuation in part of my 5 copending application, Serial No. 681,820, filed December 20th, 1923.

For a number of applications, for example, for paper manufacture, the value of clays depends upon their colour, and certain clays, 10 of which some of the Georgia clays constitute examples, have been unutilizable on account of their natural colour. The modes of treatment hitherto suggested for improving the colour of such clays have not 15 been entirely successful; and many substances which have been proposed as bleaching agents or colour improvers for clays,—oxalic acid for instance—have been found impracticable for commercial working by 20 reason of cost. As a result, most of the clays for uses in which good colour is a desideratum have been imported. The present invention has been developed with Georgia 25 clays of the type aforesaid, and has for a primary object to provide an economical means for improving the colour of these and like clays.

According to this invention, a process for 30 the treatment of clay is characterized by subjecting the clay in aqueous suspension to the action of a plurality of bleaching agents.

The clay may be treated with two or more 35 of such agents either simultaneously or successively, as may prove convenient in any given case.

I have found that a bleaching agent for 40 clay, such as oxalic acid, when used in conjunction with a co-operative bleaching agent provides a bleaching process of improved economy and efficiency. For instance, to obtain substantially the same bleaching effect 45 as that produced by a comparatively expensive reagent as oxalic acid, less of such reagent is necessary when using another suitable bleaching agent in conjunction with the acid. Moreover, by the use according to this 50 invention of a dual bleaching agent, the total quantity of reagent required to effect a given result may be less than the quantity requisite when one of the cooperative reagents alone is employed even when used more than once. There are also certain clays upon which individual reagents have no appreciable action.

For example, on some clays oxalic acid by 55 itself will not effect any material improvement in colour, nor will sodium sulphide when employed alone. When, however, these two reagents are employed in conjunction, an immediate improvement in colour is attained.

If a clay be treated with an aqueous solution of sodium sulphide, or of calcium sulphide in caustic soda, the colour of the clay becomes green or black on standing. This 60 colour is at once discharged by the strong acids, sulphuric, nitric, or hydrochloric acid, or by per-salts or hydrogen peroxide; but in nearly every case the clay returns to its original colour, and hence is still unbleached. On the other hand, if the sulphided clay be 65 treated with a reducing acid, such as oxalic acid, the green or black colouration is destroyed, the clay is bleached at the same time, and retains its improved colour after drying.

The aforesaid effects are, of course, influenced by the peculiarities of different 70 clays; for a given reagent will not necessarily act in the same way or to the same degree on different clays; but with due regard to this fact the dual reaction may be 75 said to be something more than merely additive, and a feature of the invention to reside in the treatment of clay with a plurality of bleaching agents the co-operative effect of 80 which is greater than their individual effects.

One class of co-operative reducing agents according to this invention are represented 85 by soluble salts of reducing acids, examples being salts of reducing sulphur-acids, such as, sodium sulphide, sodium sulphite, calcium sulphide in alkaline solution, sodium bisulphite, sodium oxalate, sodium metabisulphite, sodium thiosulphate, sodium hyposulphite.

The sodium salts are preferred, as, apart 90 from cost, I have found them to be more generally applicable and effective; potassium sulphide, for example, being apparently of very much more limited application than sulphide of sodium, and failing with a number of clays readily amenable to successful treatment with the latter reagent.

The other co-operative class of bleaching 95 reagents consists of acids of a reducing nature, and is exemplified by sulphurous acid and oxalic acid. Upon a number of

clays tried, formic acid was without positive result. The preferred reagent of this class is oxalic acid, by reason of its generally wide field of use and ease of application with good results.

The clay may be treated in aqueous suspension with the reducing acid, such as oxalic acid, in the presence of, or after treatment with, the co-operative reagent, the following being examples of the manner in which the invention may be carried into effect:—

*Example I.*

15 A Georgia clay from the Dry Branch District in suspension in water (20 per cent clay, 80 per cent water) was run into settling tanks prior to filter pressing in known manner. A solution in water of oxalic acid and 20 sodium thiosulphate was prepared, the proportions being about ten pounds oxalic acid and fifteen pounds sodium thiosulphate per ton of clay. This solution was run in with the clay slip as the latter passed into the 25 tanks. The clay was then allowed to settle until the bleaching was effected, which in this case required somewhat over forty-eight hours. The supernatant liquor was run off and the clay dried as usual by filter-pressing. 30 If desired the supernatant liquor after removal may be used again for the treatment of a fresh batch of clay, after suitable reinforcement with one or both of the reagents as required.

35 *Example II.*

A clay from the McIntyre District, Georgia, U. S. A., was treated, in the same way as in the preceding example, with a solution containing 16 lbs. of oxalic acid and 40 16 lbs. of 30 per cent sodium sulphide per ton of clay. After removal of the supernatant liquor the latter was re-used several times before being discarded, on adding sufficient of the cheaper ordinary sodium sulphide and hydrochloric acid to make the oxalic acid available for use again. This 45 clay remained unbleached after standing more than 24 hours on addition of 24 pounds of oxalic acid per ton of clay treated. It 50 also remained unbleached after adding 24 pounds of sodium sulphide (60%) per ton of clay treated. 15 pounds of oxalic acid per ton of clay and 30 pounds in bisulphite of soda per ton of clay will bleach this clay 55 in about 36 hours; whereas neither of these reagents alone will bleach the clay at the above mentioned concentrations.

*Example III.*

60 In like manner, a Dry Branch clay from Georgia was successfully bleached in a few days by treatment with sulphurous acid simultaneously with sulphide of sodium and sodium thiosulphate, the proportions being 65 2½ lbs. of 30 per cent sodium sulphide, 2½

lbs. of sodium thiosulphate, and 8 lbs. of commercial sulphurous acid solution per ton of clay in the form of a 20 per cent suspension.

*Example IV.*

The same clay as in Example III was treated in aqueous suspension with a solution of calcium sulphide in sodium carbonate solution, and thereafter with sulphurous acid, in the proportions of 1 lb. of calcium sulphide, 8 lbs. of sodium carbonate and 12 lbs. of a commercial solution of sulphurous acid per ton of the clay in a 20% suspension of clay in water.

It may be said that the results obtained by the use of sulphurous acid are not generally so good or so readily obtainable as when oxalic acid is employed.

In order to purify the clay and at the same time to improve its colour, the second example just described may be carried out in a different way. The sodium sulphide may be introduced alone into the clay slip, whereby the clay is deflocculated. The impurities can then be removed in known manner, and the oxalic acid solution subsequently added with a resultant improvement of colour in the course of settling. Sodium oxalate is an example of another reagent which may be employed with certain clays in order to effect purification by deflocculation as a step in the process of decolorizing.

Where the co-operative reagent used for effecting the deflocculation is one which with a particular clay displays narrow working limits of concentration, a compatible deflocculating agent may be added or used by itself alone. For instance, sodium sulphide may be employed along with sodium pyrophosphate. With some clays sodium sulphide functions as a deflocculator within inconveniently narrow limits of concentration, and in such cases this reagent may be combined with a part of the oxalic acid required for completing the bleaching effect:—

*Example V.*

One tone of a Georgia clay was mixed with four tons of water, and there were then incorporated with the mixture 2½ lbs. of 60 per cent sodium sulphide and 2¾ lbs. of oxalic acid, whereby the clay was deflocculated. After separation of the undeflocculated impurities, the remainder of the oxalic acid and sodium sulphide is added to complete the bleaching, making a total of six pounds of sodium sulphide (60%), and ten pounds of oxalic acid per ton of clay. Using 30 pounds of oxalic acid it was found that over thirty pounds of oxalic acid per ton of clay treated did not bleach the clay to any material extent after standing over thirty-six hours. Neither did 30 pounds of sodium sulphide (60%) per ton

of clay treated required to complete the bleaching process was added.

I claim:—

1. The process for the treatment of clay which comprises subjecting the clay in aqueous suspension to the action of a plurality of bleaching agents the cooperative effect of which is greater than the sum of their individual effects.
- 10 2. The process for the treatment of clay which comprises subjecting the clay in aqueous suspension to the action of a plurality of reducing agents.
- 15 3. The process for the treatment of clay which comprises subjecting the clay in aqueous suspension to the action of a plurality of reducing agents, the cooperative effect of which is greater than the sum of their individual effects.
- 20 4. The process for the treatment of clay which comprises subjecting the clay in aqueous suspension to the action of an acid of reducing properties and the sodium salt of a reducing sulphur acid.
- 25 5. The process for the treatment of clay which comprises subjecting the clay in aqueous suspension to the action of oxalic acid in co-operation with the sodium salt of a reducing acid.
- 30 6. The process for the treatment of clay which comprises subjecting the clay in aqueous suspension to the action of oxalic acid in co-operation with sodium sulphide.

7. In the treatment of clay, the steps con-

sisting of purifying the clay by deflocculation and bleaching it by a reducing agent. 35

8. In the treatment of clay, the steps consisting of purifying the clay in aqueous suspension by a deflocculator and bleaching it by a reducing agent. 40

9. In the treatment of clay, the steps consisting of deflocculating the clay in aqueous suspension by an alkali deflocculator and then bleaching it by a reducing agent.

10. The process for the treatment of clay which comprises subjecting the clay in aqueous suspension to the simultaneous action of oxalic acid and sodium sulphide. 45

11. The process for the treatment of clay which comprises deflocculating the clay as 50 a step in the bleaching thereof by initially treating the clay in aqueous suspension with a co-operative bleaching reagent of deflocculating property and, after removal of any undeflocculated impurities, treating the clay 55 suspension with another cooperative bleaching reagent to complete the bleaching.

12. The process for the treatment of clay which comprises deflocculating the clay as a 60 step in the bleaching thereof by initially treating the clay in aqueous suspension with sodium sulphide and, after removal of any undeflocculated impurities, treating the clay suspension with oxalic acid.

In testimony whereof I affix my signature. 65

WILLIAM FELDENHEIMER.